

## 1

3,573,225

**RUST-PROOFING COMPOSITE SOLUTIONS**  
 Masahiko Kondo, 3-14-7 Maechi, Saitama Prefecture,  
 Urawa, Japan, and Tetsuo Shimmura, 27 Futaba-cho,  
 Itabashi-ku, Tokyo, Japan  
 No Drawing. Filed Feb. 1, 1968, Ser. No. 702,209  
 Int. Cl. C23f 11/14, 11/10  
 U.S. Cl. 252—392

6 Claims

**ABSTRACT OF THE DISCLOSURE**

Rust-proofing aqueous or alcoholic composite solutions for application to metal surfaces consisting essentially of an amine salt of a fatty acid, an alkali metal salt of benzoic acid and an alkanolamide.

This invention relates generally to rust-proofing compositions for application to metal surfaces and has particular reference to such aqueous or alcoholic composite solutions which consist essentially of an amine salt of a fatty acid, an alkali metal salt of benzoic acid and an alkanolamide.

There are known a variety of rust preventives useful for protecting metal surfaces against corrosion attack, most widely used of which is an oil-film forming material. This material also varies in kind, and although some are better than the others in terms of the length of time in which they retain rust-proofing efficacy, they are all adequate for all practical purposes.

However, these unctuous rust preventives are difficult to remove from the metal surfaces to which they have been applied. This film removal operation is time-consuming and troublesome, requiring the use of an alkali solution or chlorinated solvents such as trichloroethylene and perchloroethylene with which to wash the film off sometimes with heating, or sometimes using petroleum series solvents.

To eliminate such difficulty, there have more recently been introduced certain water-soluble rust-proofing compositions which need not be removed after deposit on the metal surfaces or may be removed with ease. Typical examples are an alkali metal nitrite, dicyclohexylammonium nitrite, cyclohexylammonium nitrite and an alkali metal chromate. These aqueous solutions have been found useful insofar as the metal is soaked therein, but they are not quite as effective as oil counterparts when applied to the metal surfaces and exposed to the outside atmosphere for extended periods of time.

It is the primary object of the present invention to provide new, useful rust-proofing or rust-preventive compositions of this character which have prolonged efficacy in protecting metal surfaces against corrosion and which can be removed therefrom with utmost ease as the occasion calls for.

It is another object of the invention to provide rust-proofing compositions which, on application to metal surfaces, will form a transparent or translucent uniform film thereby retaining the original surface appearance of the metal.

Briefly stated, the inventive concept of the present invention resides in the peculiar combination of an amine salt of a fatty acid, an alkali metal benzoate and an alkanolamide whereby there is obtained a highly effective, long-lasting rust preventive product. It has been empirically ascertained that the absence of any one of the three compounds or any one thereof alone cannot achieve the desired characteristics of the rust preventives comparable to, or better than existing oil type counterparts.

An amine salt of a fatty acid having a certain range of molecular weight is known as a volatile rust preventive

## 2

compound which tends to sublimate at room temperature.

An alkali metal benzoate is known as a contact rust preventive compound useful for coating on metal surfaces, and it may be added with a corrosive solution to make the most of its rust-preventive tendency.

5 An alkanolamide has both surface-active and contact rust-preventive properties. This surface-active agent helps reduce the surface tension of the composite solution when applied to metal surfaces, so that the contact rust-preventive tendency of the solution is so much increased.

10 It has been discovered that an amine salt of a fatty acid, e.g. cyclohexylamine laurate, and an alkali metal benzoate, e.g. sodium benzoate, are highly conducive to the rust-preventive life time, while an alkanolamide

15 co-present in the composite solution serves to reduce the surface tension thereof, so as to facilitate its deposit on metal surfaces. Experiments show that the rust-proofing composite solution according to the invention will form on the metal surface a uniform film about 0.005 to 5 20 microns thick after the water or alcoholic contents thereof have evaporated.

25 There are different theories to account for the mechanism in which organic corrosion-inhibitors exhibit their rust-proofing activity on metal surfaces. One theory is based on the physical adsorption of the inhibitor to the metal surface. Another theory is based on the chemical adsorption. Still another theory attributes it to the formation of a chelate compound.

30 With an organic corrosion-inhibitor dissolved in water, alcohol or benzene, for application to metal surfaces, it would be useless, were it not for a deposit of adequate amounts of the inhibitor on the metal surfaces, even if there has been formed a chelate compound which would necessarily be only appreciable and susceptible to destruction by ambient causes.

35 On the other hand the alkanolamide included in the composite rust-preventive composition according to the present invention has a peculiar surface-active effect to permit the amine salt of a fatty acid and the alkali metal benzoate to deposit on metal surfaces in an amount greater than required for chemical adsorption, although it does not possess as great corrosion-inhibitive activity as the latter two compounds.

40 Experiments revealed that the best results are obtainable by blending 50–100 parts by weight of amine salt of fatty acid, 20–200 parts of alkali metal benzoate, and 1–50 parts of alkanolamide to 0.5–20% consistency in an aqueous or alcoholic solution. Blends in excess of the upper limit of this range were found commercially 45 unfeasible, and those less than the lower limit inoperative. More specific blending proportions will be discussed in the examples given hereinafter.

45 The term, amine salt of fatty acid according to the invention includes reaction products of a saturated fatty acid having a carbon number of 6–18 with an alkyl- or cycloalkyl-amine having a carbon number of 6–12, for example, cyclohexylamine laurate, dicyclohexylamine caprylate, cyclohexylamine myristate and octylamine stearate. The saturated fatty acid and the amine are reacted in a mol ratio equivalent to each other, or with a slight excess of the latter, the resulting product being in the form of a salt free of amide bonds.

50 The term alkali metal benzoate includes sodium benzoate, potassium benzoate and lithium benzoate. Instead of the alkali metal benzoate, nitrite compounds such as sodium nitrite may be used.

55 The term alkanolamide includes reaction products of a fatty acid having a carbon number of 6–18 with N-hydroxyethyl or N,N-bis-hydroxyethyl capramide, N-hydroxyethyl or N,N-bis-hydroxyethyl oleamide; or N-hydroxyethyl or N,N-bis-hydroxyethyl lauramide. 1 mol of such

fatty acid is reacted with 2 mols of the alkanolamide, so that the excess of the latter loosely combines with the resulting amide thereby affording enhanced water-solubility.

The rust-preventive compositions according to the invention may be applied to iron, alloys thereof, aluminum, tin, zinc, and other metals. This may be done by the use of brush, rolls, sprayers, or otherwise by dipping the metal in the composite of the invention.

#### EXAMPLE 1

There were prepared three different aqueous solutions: the first was a composite aqueous solution of cyclohexylamine laurate, N,N-bis-hydroxyethyl lauramide, and sodium benzoate; the second was a composite aqueous solution of any two of the above three compounds; and the third was a mono aqueous solution of any one of the above three compounds, as tabulated below.

TABLE 1

|                                             | Compounds                           | Amounts by weight | Corrosion-inhibitive factor (percent) | 25 |
|---------------------------------------------|-------------------------------------|-------------------|---------------------------------------|----|
| Sample 1...                                 | Cyclohexylamine laurate.....        | 100               |                                       |    |
|                                             | N,N-bis-hydroxyethyl lauramide..... | 10                | 100                                   |    |
|                                             | Sodium benzoate.....                | 100               |                                       |    |
|                                             | Water.....                          | 3,000             |                                       |    |
| Sample 2...                                 | Cyclohexylamine laurate.....        | 150               |                                       |    |
|                                             | N,N-bis-hydroxyethyl lauramide..... | 60                | 75                                    | 30 |
|                                             | Water.....                          | 3,000             |                                       |    |
|                                             | Cyclohexylamine laurate.....        | 150               |                                       |    |
| Sample 3...                                 | Sodium benzoate.....                | 60                | 90                                    |    |
|                                             | Water.....                          | 3,000             |                                       |    |
|                                             | N,N-bis-hydroxyethyl lauramide..... | 150               |                                       |    |
|                                             | Water.....                          | 3,000             |                                       |    |
| Conventional oil type rust preventives..... | Cyclohexylamine laurate.....        | 210               |                                       |    |
|                                             | Water.....                          | 3,000             | 80                                    | 35 |
|                                             | N,N-bis-hydroxyethyl lauramide..... | 210               |                                       |    |
|                                             | Water.....                          | 3,000             |                                       |    |
| Untreated steel.....                        | Sodium benzoate.....                | 210               | 70                                    |    |
|                                             | Water.....                          | 3,000             |                                       |    |
| Commercial oil type rust preventives.....   |                                     | 85                |                                       |    |
| Untreated steel.....                        |                                     | 95                |                                       |    |
| Untreated steel.....                        |                                     | 20                |                                       |    |

Note.—Corrosion-inhibitive factor is represented by rust-free surface area/test piece surface area  $\times 100$ .

A test piece of cold-roll steel measuring 60 mm. x 80 mm. x 1.2 mm. was immersed in each sample solution and immediately taken out for exposure to the atmosphere for about 30 minutes, until a film of this solution about 0.7 micron thick was formed on the surfaces of the test piece. The test piece thus treated was packed in a polyethylene laminated paper but unsealed to permit aeration.

Commercially available rust preventives of the oil type also participated in this test under similar conditions, for

purposes of comparison. Each packed test piece was placed in a 60° C., 90% relative humidity constant temperature container and disposed thus for 15 consecutive days, with the results given in Table 1.

#### EXAMPLE 2

Three different sample solutions were prepared in a manner similar to Example 1, using dicyclohexylamine caprylate, N-hydroxyethyl oleamide and sodium benzoate.

10 Water and methanol were used as solvent. The same test piece as in Example 1 was treated in similar conditions to obtain on its surface 0.6 micron thick film of the solution. Each packed test piece was disposed for 15 days in a constant temperature container cycling every 16 hours with a set of conditions of 60° C. and 80% relative humidity and every 8 hours with another set of conditions of 5° C. and 80% relative humidity. Commercially available oil-type counterparts similarly participated in this test. Test results are shown in Table 2.

TABLE 2

|                                             | Compounds                                   | Amounts by weight | Corrosion-inhibitive factor (percent) |
|---------------------------------------------|---------------------------------------------|-------------------|---------------------------------------|
| Sample 1...                                 | Dicyclohexylamine caprylate.....            | 100               |                                       |
|                                             | N-hydroxyethyl oleamide.....                | 20                |                                       |
|                                             | Sodium benzoate.....                        | 100               | 100                                   |
|                                             | Water.....                                  | 1,500             |                                       |
| Sample 2...                                 | Methanol.....                               | 1,500             |                                       |
|                                             | Dicyclohexylamine caprylate.....            | 200               |                                       |
|                                             | N-hydroxyethyl oleamide.....                | 20                |                                       |
|                                             | Water.....                                  | 1,500             | 70                                    |
| Sample 3...                                 | Methanol.....                               | 1,500             |                                       |
|                                             | Dicyclohexylamine caprylate.....            | 110               |                                       |
|                                             | Sodium benzoate.....                        | 110               |                                       |
|                                             | Water.....                                  | 1,500             | 85                                    |
| Conventional oil type rust preventives..... | Methanol.....                               | 1,500             |                                       |
|                                             | Dicyclohexylamine caprylate.....            | 220               |                                       |
|                                             | Water.....                                  | 1,500             | 60                                    |
|                                             | Methanol.....                               | 1,500             |                                       |
| Untreated steel.....                        | N-hydroxyethyl oleamide.....                | 220               |                                       |
|                                             | Water.....                                  | 1,500             | 40                                    |
|                                             | Methanol.....                               | 1,500             |                                       |
|                                             | Sodium benzoate.....                        | 220               |                                       |
| Conventional oil type rust preventives..... | Water.....                                  | 1,500             | 75                                    |
|                                             | Methanol.....                               | 1,500             |                                       |
|                                             | Conventional oil type rust preventives..... | 1,500             | 80                                    |
|                                             | Untreated steel.....                        | 5                 |                                       |

45 Note.—Corrosion-inhibitive factor is represented by rust-free surface area/test piece surface area  $\times 100$ .

#### EXAMPLE 3

50 Example 2 was followed, except for the use of pure aluminum measuring 60 mm. x 8 mm. x 2 mm. as a test piece. Corrosion of the test piece was determined by comparing the surface condition of the test piece prior to treatment with that after treatment.

TABLE 3

|                          | Compounds                        | Amounts by weight | Surface condition            |
|--------------------------|----------------------------------|-------------------|------------------------------|
| Sample 1...              | Dicyclohexylamine caprylate..... | 100               |                              |
|                          | N-hydroxyethyl oleamide.....     | 20                |                              |
|                          | Sodium benzoate.....             | 100               | Unchanged.                   |
|                          | Water.....                       | 1,500             |                              |
| Sample 2...              | Methanol.....                    | 1,500             |                              |
|                          | Dicyclohexylamine caprylate..... | 200               |                              |
|                          | N-hydroxyethyl oleamide.....     | 20                |                              |
|                          | Water.....                       | 1,500             |                              |
| Sample 3...              | Methanol.....                    | 1,500             | Partly white spot rust.      |
|                          | Dicyclohexylamine caprylate..... | 110               |                              |
|                          | Sodium benzoate.....             | 110               |                              |
|                          | Water.....                       | 1,500             |                              |
| Untreated aluminium..... | Methanol.....                    | 1,500             |                              |
|                          | Dicyclohexylamine caprylate..... | 220               |                              |
|                          | Water.....                       | 1,500             |                              |
|                          | Methanol.....                    | 1,500             | Partly white spot rust.      |
| Untreated aluminium..... | N-hydroxyethyl oleamide.....     | 220               |                              |
|                          | Water.....                       | 1,500             |                              |
|                          | Methanol.....                    | 1,500             |                              |
|                          | Sodium benzoate.....             | 220               |                              |
| Untreated aluminium..... | Water.....                       | 1,500             |                              |
|                          | Methanol.....                    | 1,500             |                              |
|                          | Water.....                       | 1,500             |                              |
|                          | Methanol.....                    | 1,500             | White rust in total surface. |

## EXAMPLE 4

The various sample solutions listed in Table 4 below were prepared, 100 cc. of each of which were placed in a container measuring 9 cm. in inside diameter and 15 cm. in height. A test piece of cold-roll steel measuring 6 cm. x 10 cm. x 0.2 cm. was introduced halfway into the container, and disposed thus for 30 consecutive days, with the upper half portions of the test piece exposed to the atmosphere. A blank test was also conducted with use of distilled water.

a fatty acid selected from the group consisting of the reaction products of amines having 6-12 carbon atoms and a saturated fatty acid having 6-18 carbon atoms, 20-200 parts by weight of an alkali metal benzoate, 1-50 parts by weight of an alkanolamide selected from the group consisting of the reaction products of ethanolamines and a saturated fatty acid having 6-18 carbon atoms, and a mixture of alcohol and water in an amount to produce an 0.5-20% alcohol solution.

5. A rust-proofing composite solution as claimed in 10 claim 4, wherein the alkali metal benzoate is selected

TABLE 4

| Compounds            | Amount<br>by weight          | Corrosion-inhibitive<br>factor (percent) |                    |
|----------------------|------------------------------|------------------------------------------|--------------------|
|                      |                              | Immersed<br>portion                      | Exposed<br>portion |
| Sample 1-----        | Caprylamine laurate.....     | 120                                      | 100                |
|                      | N-hydroxyethyl oleamide..... | 20                                       |                    |
|                      | Sodium benzoate.....         | 180                                      |                    |
|                      | Water.....                   | 3,000                                    |                    |
| Sample 2-----        | Caprylamine laurate.....     | 320                                      | 80                 |
|                      | Water.....                   | 3,000                                    |                    |
|                      | N-hydroxyethyl oleamide..... | 320                                      |                    |
|                      | Water.....                   | 3,000                                    |                    |
| Distilled water..... | Sodium benzoate.....         | 320                                      | 40                 |
|                      | Water.....                   | 3,000                                    |                    |
| Distilled water..... |                              | 100                                      | 60                 |
|                      |                              | 0                                        | 5                  |

NOTE.—Corrosion-inhibitive factor is represented by rust-free surface area/test piece surface area  $\times 100$ .

## What is claimed is:

1. A rust-proofing composite solution consisting essentially of 50-100 parts by weight of an amine salt of a fatty acid selected from the group consisting of the reaction products of amines having 6-12 carbon atoms and a saturated fatty acid having 6-18 carbon atoms, 20-200 parts by weight of an alkali metal benzoate, 1-50 parts by weight of an alkanolamide selected from the group consisting of the reaction products of ethanolamines and a saturated fatty acid having 6-18 carbon atoms, and water in an amount to produce an 0.5-20% aqueous solution.

2. A rust-proofing composite solution as claimed in claim 1, wherein the alkali metal benzoate is selected from the group consisting of sodium benzoate, potassium benzoate and lithium benzoate.

3. A rust-proofing composite solution as claimed in claim 2, wherein the amine salt of a fatty acid is selected from the group consisting of cyclohexylamine laurate, dicyclohexylamine caprylate, cyclohexylamine myristate and octylamine stearate, and said alkanolamide is selected from the group consisting of N-hydroxyethyl oleamide, N,N-bis-hydroxyethyl capramide and N,N-bis-hydroxyethyl lauramide.

4. A rust-proofing composite solution consisting essentially of 50-100 parts by weight of an amine salt of

from the group consisting of sodium benzoate, potassium benzoate and lithium benzoate.

6. A rust-proofing composite solution as claimed in 30 claim 5, wherein the amine salt of a fatty acid is selected from the group consisting of cyclohexylamine laurate, dicyclohexylamine caprylate, cyclohexylamine myristate and octylamine stearate and said alkanolamide is selected from the group consisting of N-hydroxyethyl oleamide, N,N-bis-hydroxyethyl capramide and N,N-bis-hydroxyethyl lauramide.

## References Cited

## UNITED STATES PATENTS

|           |        |                |       |         |
|-----------|--------|----------------|-------|---------|
| 2,739,870 | 3/1956 | Senkus         | ----- | 252—392 |
| 2,782,164 | 2/1957 | Fischer et al. | ----- | 252—392 |
| 2,850,461 | 9/1958 | Bloch et al.   | ----- | 252—394 |

45 RICHARD D. LOVERING, Primary Examiner

I. GLUCK, Assistant Examiner

U.S. CL. X.R.

50 21—2.7; 252—390, 296